

# UNITED STATES PATENT OFFICE.

ALBERT W. SPERLING, OF INDEPENDENCE, OREGON.

## PROCESS OF IMPRESSING TYPE OF A TYPEWRITING-MACHINE DIRECTLY INTO THE MOLD FOR MAKING STEREO TYPE.

1,366,032.

Specification of Letters Patent. Patented Jan. 18, 1921.

No Drawing.

Application filed March 18, 1919. Serial No. 283,432.

To all whom it may concern:

Be it known that I, ALBERT W. SPERLING, a citizen of the United States of America, (whose post office address and place of residence is at Independence, Oregon,) have invented a new and useful Improvement in Processes of Impressing Type of Typewriting-Machines Directly into the Mold for Making Stereotype.

10 Heretofore molds for making stereotype therefrom have been made by impressions taken from a group of movable type; these type have been set up either by hand or by complicated mechanical contrivances.

15 An object of the invention is to provide a simple and economical process whereby an expert typist can be employed instead of a type setter, it being possible for one typist to do work which by any other method 20 would require the employment of two or more type setters. A further object is to eliminate the necessity of sorting type, as where ordinary hand methods of type setting are employed.

25 To carry my invention into effect I take a piece of thin blotting paper and from this I prepare my mold as follows:

I place this blotting paper in a bath or solution made of 3 parts of (commercial) 30 sodium silicate and one part of water and leave it soak till it is thoroughly soaked through with the solution which requires about ten minutes.

35 I then take the piece of blotting paper and press out all the surplus liquid by running it through a rubber roller clothes wringer, with a slight pressure on the rollers and removing all surplus liquid, or that which appears glossy after this, with a dry 40 piece of blotting paper, for any surplus liquid on the mold will clog the type on the typewriting machine.

45 I then take a thicker piece of dry blotting paper and soak this in a bath of glycerin and press out all the surplus glycerin by running it through the wringer.

50 I then take this piece of blotting paper (soaked in the glycerin) and place it face to face with the blotting paper soaked in the sodium silicate and water bath, and press the two together by running them through the wringer, after this I separate them. The object of this is to distribute just enough glycerin or oil on the face of the 55 mold to keep the sodium silicate from clog-

ging the type on the typewriting machine and also prevent sticking thereof.

I then remove the ink pad or carbon inked ribbon from the typewriting machine and start a small piece of thin paper, say 4 by 6 inches, through the typewriting machine and underneath this, say about one inch from the end of the thin paper, I start my blotting paper, soaked in the sodium silicate and water bath, through the typewriting machine. The object of this is to start the blotting paper through the typewriting machine without doubling up the blotting paper. After the blotting paper is started in the typewriting machine it passes 65 through like any ordinary writing paper.

I then proceed to type write on the blotting paper, soaked in the sodium silicate and water bath, and press a trifle harder on the keys of the typewriting machine than I 70 would for ordinary typewriting. The type of the typewriting machine will impress or perforate the blotting paper, soaked in the sodium silicate and water bath, to the extent of all but a thin film that is left on the 75 bottom of the blotting paper, just thick enough to hold the impression of the type face of the typewriting machine, and not allow the lead to run through the mold when the stereotype is cast from the mold.

80 After this the blotting paper or mold as it is now called is carefully removed from the typewriting machine and placed on a warmer of a temperature of about 125 degrees, for a few minutes. The object of this 85 is to set the sodium silicate in the mold and prevent it from sticking when placed between the plates for baking.

I now place the mold between two cast iron plates with a slight pressure thereon, 90 and bake it at a low heat until the mold is of a deep ochre color. Then I remove the mold.

95 The cast iron plates must be smooth and absolutely true or the type will not be all 100 of uniform height. After the mold is removed from the cast iron plates I proceed to build it up with a compound in order to keep the printing press ink rollers from striking the barren or unlettered parts of the stereotype cast from the mold, which I do as follows:—I take one part of dry flaked glue to about 35 parts of refined whiting by weight, after the glue is dissolved in boiling water, I mix it with the whiting (grinding it 105 110

smooth) and thin it with water until the compound is of the right flowing consistency; to flow well and yet not run.

I then strain the compound through a piece of cheese cloth and then I put the compound in an air pencil or relief bulb, which is a rubber bulb with a spout attached to the same. I then proceed to flow this compound on the mold with the air pencil between the 10 impressed lines and words of type and the majority of the space that is not impressed with the type, using a smaller air pencil and a thinner compound between the impressed words and lines of the impressed type, and 15 a larger air pencil and a thicker compound on the margin and the large vacant spaces that is not impressed with the type, thereby enabling me to build up the large vacant spaces considerably higher on the mold with 20 the thicker compound. After the compound on the mold has dried sufficiently on a warmer to prevent sticking, I replace the mold between the cast iron plates and reheat at a low temperature, laying a thin sheet of 25 paper and a thin layer of cotton batting on the face of the mold to insure a smooth and level mold, and place a slight pressure thereon, and when the moisture is dried out of the compound and the mold, I remove it 30 from the cast iron plates, and the mold is then ready for the stereotype caster. If the mold sticks to the stereotype from slight moisture being therein, the stereotype is placed in hot water till the mold and compound comes off of the stereotype, after 35 which the stereotype is ready for the printer. The sodium silicate acts as a three fold agent, viz:—1st. It softens the blotting paper so that the type from the typewriting 40 machine will penetrate it all but a thin film of the paper, just thick enough to hold the impression of the type. 2nd. It makes the blotting paper hold its shape to the form of the imprint of the type; not allowing the 45 imprint to spring back or out of shape. 3rd. It hardens the blotting paper or mold, after it is placed between the plates for baking, making it easy to handle and making a kind of fireproofing for the mold while baking it. When this process is used on such 50 typewriting machines as the Blickens- derfer, and other makes of typewriting machines with a type wheel, or interchangeable type thereon, rapid changes can be made in

different sizes and styles of type, thereby 55 giving the printer an almost unlimited variety of different kinds and styles of type to select from.

I do not claim the invention of any type-writing machine or tools or any mechanical 60 improvement thereon, that I use with my process.

What is claimed is:—

1. The herein described step in the process of producing stereotype molds which consists in saturating a sheet of blotting paper with a solution of sodium silicate, then removing surplus solution by pressure, and then applying thereto a sheet of blotting paper containing glycerin and subjecting 65 the two sheets to pressure to transfer a film of glycerin to the sheet containing sodium silicate.

2. The herein described step in the process of producing stereotype molds which consists in saturating blotting paper with a solution of sodium silicate and then pressing surplus solution therefrom, then applying to the sheet a coating of glycerin or the like, and then forming in a surface of the sheet 70 impressions of the type of a typewriting machine or the like.

3. The herein described process of producing stereotype molds which consists in impregnating a sheet of blotting paper or the 75 like with a solution of sodium silicate, removing surplus solution from the sheet, applying glycerin to the surface of the sheet, forming in the face of the sheet impressions of type, then drying the mold and baking it 80 between smooth plates holding it under pressure.

4. The herein described process of producing stereotype molds which consists in baking between smooth surfaces a sheet of blotting paper or the like containing type impressions and which has been saturated with sodium silicate solution and surfaced with glycerin, then removing the mold from between said surfaces and building up thereon 95 between the impressions with a mixture of glue and whiting.

ALBERT W. SPERLING.

Witnesses:

CLIFFORD MCBEATH,  
C. O. SLOPER,  
J. G. MCINTOSH.